

## UNITED STATES PATENT OFFICE

2,325,840

METHOD OF WATERPROOFING FUEL  
BRIQUETTES

John A. Erickson, Jackson, Mich.

No Drawing. Application April 4, 1941,  
Serial No. 386,839

2 Claims. (Cl. 44—10)

The present invention relates to fuel briquettes and more particularly to a method of waterproofing fuel briquettes manufactured from a finely divided fuel using a starch base binder.

The present application is a continuation in part of my copending application Serial No. 272,490, filed May 8, 1939, and particularly contemplates waterproofing briquettes made according to the invention disclosed in said copending application. It is to be understood, however, that the present invention contemplates the waterproofing of any briquette regardless of the method by which they are made. However, briquettes made with a binder of such materials as asphalt, pitches, tars, and the like, do not need waterproofing and therefore as a commercial proposition the waterproofing of briquettes made with such binders ordinarily would not be undertaken by the present method.

According to the present invention, briquetting material of finely divided fuel and a suitable binder is thoroughly mixed and prior to molding in briquettes is subjected to a finely divided spray of a hydrocarbon, solid at ordinary temperatures but liquefiable at elevated temperatures. The atomized hydrocarbon is permitted to solidify before striking the briquetting mixture. Then the finely divided particles are thoroughly mixed with the briquetting mixture and the mixture molded to provide briquettes. The temperature of the briquettes is then elevated to fuse the finely divided hydrocarbon particles to waterproof the briquettes.

An object of the present invention is to waterproof briquettes made with a non-waterproof binder.

Another object of the invention is to waterproof briquettes made with a starch base binder.

Still another object of the invention is to waterproof briquettes by spraying onto the briquetting material prior to molding a combustible solid, fusible at elevated temperatures, and subsequent to molding the briquettes, elevating the temperature of the briquettes to fuse the combustible solid.

A still further object of the invention is to waterproof briquettes made with a non-waterproof binder by mixing it with a finely divided hydrocarbon which is solid at ordinary temperatures and then elevating the temperature of the molded briquettes to fuse the hydrocarbon.

These and other objects will be apparent from the following specification wherein my invention is described in detail:

The present invention may be employed in the

waterproofing of briquettes made from substantially any briquettable fuel. For the purpose of fully disclosing my invention I will disclose generally the method of making briquettes according to my above identified parent application.

The invention disclosed and claimed in my above identified application may be employed in the production of briquettes from substantially any of the briquettable fuels. In the case of semi-anthracite fines a starch binder according to said invention may be employed as the sole binding agent. However, it is contemplated that in the manufacturing of briquettes according to said invention, other materials not specifically related to the present invention such as coking coals, for example, may be employed when required. For instance, in the case of coke breeze and petroleum coke fines it is often necessary to add a low-volatile strongly coking coal due to the porous nature of the coke which otherwise would absorb a large quantity of binder, and due to the fact that the addition of such coal results in a briquette which does not so readily disintegrate in a fire. When employing anthracite fines the addition of a strongly coking coal is required to prevent disintegration during burning. In other cases, such as in certain types of bituminous coal, lignites, etc. it is often necessary to add an additional binder such as a cement, a tar, a resin, an asphalt, or another known binder. In the present disclosure it is considered that fuel or briquettable fuel contemplates fuel in a briquettable state, either with or without the addition of a material necessary for practical reasons to make the fuel briquettable and bindable with a starch adhesive.

While any starch may be employed, it is preferred that starch from grain and tubers, such as potatoes and yams, be employed as these raw materials are readily available. Inasmuch as the process permits the use of cheap grain, old potatoes, or starch bearing roots and the like, which have become moldy or otherwise unfit for their usual consumption, this type of a source for starch is recommended. In obtaining starch from the materials herein specified, no refinement is necessary. In each case the whole source of starch may be finely divided in manners known in the art, and the resulting product used directly.

Approximately equal parts by volume of starch in a dry finely divided form ad water are mixed together and to the mixture is added a caustic. When the starch is in the form of crushed tubers or the like containing a relatively large amount

of water, it is to be understood that the amount of water added must be based on the volume of dry starch, and that therefore in such cases it may not be necessary to add any additional water. In fact it may be necessary to remove some water. While any caustic may be employed, practical considerations require that the caustic actually used be sufficiently strong in order not to require too much of it to provide the results desired. Furthermore, economy requires that the caustic employed be relatively inexpensive. From these considerations, at the present time, sodium hydroxide and sodium carbonate are the most desirable. However, it will be understood that other caustics may be employed if desired. These caustics may be used either separately or in combination. In the case of sodium hydroxide, used alone, approximately 2% by volume of the dry starch should be added to the mixture of starch and water. In the case of other caustics, the percentage thereof employed will depend on the strength of the caustic used. The entire mixture then is agitated vigorously at a temperature approximately from 190 to 200° F. for a period of about 30 minutes. The temperature may be readily controlled by employing a steam jacketed mixer.

The temperature and agitation plus the action of the caustic convert the starch into a binder of maximum adhesive properties, although the use of heat and agitation are only for the purpose of speeding up the action of the caustic. Ordinary starch is insoluble to any substantial extent in water due to the existence of an inert insoluble coating resembling cellulose in structure which surrounds each of the starch granules. The caustic has the effect of weakening this cellulose-like coating permitting the granules to burst to free the starch. The starch is then dissolved in the water of the mixture, the dissolving being assisted by the action of the heat and the agitation. At the same time the caustic reacts with a portion of the starch to produce dextrine and dextrose, both of which are water soluble and dissolve. While it is not known exactly the relative percentages of the starch, dextrine and dextrose in the resulting mixture, it is believed that approximately 15 to 20% of the starch remains in solution. It is known, however, that substantial percentages of dextrine and dextrose are obtained. The original starch is now reduced to a form where it has its maximum adhesive properties.

In actual practice it has been found by experiments that the binder reaches its point of maximum adhesiveness when it becomes substantially transparent. Substantial transparency may be determined by placing a small quantity of the binder on a piece of glass and holding it before a source of light. At this point, the starch granules have completely dissolved and a part of the dissolved starch has been converted into dextrine and dextrose. The period of time required for preparing the binder, the temperature, the amount of agitation, and the percentage of caustic employed may all be varied as desired and as required so long as the resulting product is in the substantially transparent form described. While as explained above, the strength of the caustic employed will have a bearing on the percentage thereof required, the percentage required will also vary depending on the character of the starch employed, as well as on the temperature and time. Thus, for example, in using a temperature of from 190 to 200° F. as in the

above example, but a greater percentage of sodium hydroxide than 2% of the dry weight by volume of the starch, the time for completely preparing the binder will be reduced. Conversely should the time be increased, while retaining the same temperature, the percentage of caustic employed may be reduced. Further, if the percentage of caustic is retained at 2% of the dry weight of the starch and the temperature reduced, the time will have to be increased. As an example, with approximately 2% of sodium hydroxide by volume of the weight of the dry starch and the temperature of the mixture at approximately 220° F. a cooking for 10 minutes will convert the mixture into a binder having maximum adhesive properties. In order to raise the cooking temperature above 190 to 200° F., it will of course be necessary to heat the mixture under pressure. It should be observed that the temperature at which the mixture is maintained during the treatment should not be permitted to raise to such an extent as to caramelize the dextrine or dextrose, as the caramel is extremely inferior as a binding agent.

During the initial period of heating and agitating the complete mixture, the mass of material becomes very thick due to the absorption of the water by the starch granules. However, during the latter stages of the heating and agitating, the mixture is converted into a semi-fluid mass. This conversion is the result of the dissolving of the starch in the water following the action of the caustic on the coating surrounding each starch granule, and on the conversion of a portion of the starch into dextrine and dextrose. It will thus be apparent that there is obtained a highly efficient adhesive with a relatively small quantity of water. This result is far more satisfactory than the inefficient adhesive obtained embodying a relatively large quantity of water obtained when the starch is merely added to water and heated in the manner of the prior art.

When the semi-fluid mass of dissolved starch, dextrine and dextrose has been prepared in the manner hereinabove set forth, it is mixed with fuel fines in suitable mixing apparatus. It is preferred that the briquette material be heated during mixing so that after the briquettes have been formed their heat will expedite drying. In the case of semi-anthracite fines the binder used should contain about  $\frac{1}{2}$  to 2% by weight of dry starch of the weight of the coal fines, depending on the nature of the coal and on the hardness desired in the finished briquette. It will be understood that other types of briquettable fuel may require a greater or lesser percentage of binder, depending on the nature of the fuel and on the adhesive characteristics of materials that may be added to them. When the fuel and binder have been mixed, the briquette mixture is formed into briquettes in any known or desirable manner.

Should the fuel fines, which are to be converted into briquettes, come directly from a washing plant or from storage where they have accumulated an excessively large amount of moisture, it may be necessary to remove some of the moisture by evaporation before or after mixing with the binder. The amount of moisture, however, has no detrimental effect on the briquettes either as to strength or otherwise but may prolong the hardening of the briquettes an unreasonable length of time. The amount of moisture present in the coal, however, may be detrimental if the briquettes are to be wrapped in paper or placed in paper bags, for the reason that the moisture in the briquettes may excessively soften the

paper. On the other hand, if fuel to be briquetted is too dry it may be necessary to add water with the binder. Thus a mixture of fuel fines and a binder may be reduced to a briquettable state by only mixing or it may be necessary to add or to remove water as well as to mix the ingredients.

When the molded briquettes are to be stored in a damp basement or in a place where they might accumulate mold, the fuel and binder mixture may have added to it some antiseptic ingredient such as copper sulphate or sodium fluoride in proportions well known in the art.

In order to waterproof briquettes made according to the above method, a waterproofing agent is added to the mixture of binder and fuel fines while they are still in the mixing machine and under motion. As a waterproofing agent, a heavy hydrocarbon such as paraffin wax or a high melting point asphalt is atomized while hot and under pressure, through a nozzle, to divide it into minute globules. These minute globules are directed at the moving mixture of coal and binder while in the mixing machine. The atomizing nozzle should be placed several inches away from the moving coal and binder mixture, in order to permit the minute particles of waterproofing material to harden before they strike the briquette mixture. These hardened minute particles, striking the briquette mixture, are thoroughly mixed with it while still retaining their individual state of finely divided particles.

The briquetting mixture treated with the waterproofing material is then formed in a known or desired manner into briquettes, the temperature being kept below the melting point of the waterproofing material. After being formed into briquettes, the moisture in the briquettes is driven off at a temperature below the melting point of the waterproofing material. In order to drive off the moisture, any standard or desired drying equipment may be employed. After the moisture has been removed, during which removal the starch binder has become hardened, the temperature of the briquette is raised above the melting point of the waterproofing material, causing the waterproofing material to fuse and seal all of the pores in the briquette with a water repellent material. This water repellent material also serves to increase the strength of the briquette.

It will be understood that when employing the waterproofing method according to the present invention, the waterproofing material may be

directed on to and mixed with other briquetting mixtures, prior to molding into briquettes, than the one specifically disclosed. Furthermore, it is contemplated that the invention not be limited to the use of a combustible hydrocarbon solid at ordinary temperatures. For instance, any other material having the same functional characteristics as the hydrocarbon disclosed could be employed.

Having thus described my invention, what I desire to secure by Letters Patent and claim is:

1. The method of waterproofing solid fuel briquettes having a starch binder which comprises heating a hydrocarbon, solid at ordinary temperatures, to a temperature to permit atomizing, atomizing the hydrocarbon in a finely divided spray, directing the atomized hydrocarbon onto a briquette mixture prior to briquetting while in motion in a mixing machine, while requiring the atomized hydrocarbon to pass through the atmosphere a sufficient distance to permit the same to solidify into finely divided particles before striking the briquette mixture, whereby the finely divided particles are mixed with the briquetting material, forming the briquetting material into briquettes at a temperature below the melting point of the hydrocarbon, heating the briquettes at a temperature below the melting point of the hydrocarbon, and raising the temperature of the briquettes above the melting point of the hydrocarbon to melt the finely divided particles of the hydrocarbon in the briquettes to waterproof the same.

2. The method of waterproofing solid fuel briquettes having a starch binder which comprises heating a hydrocarbon, solid at ordinary temperatures, to a temperature to permit atomizing, atomizing the hydrocarbon in a finely divided spray, directing the atomized hydrocarbon onto a briquette mixture prior to briquetting while in motion in a mixing machine, while requiring the atomized hydrocarbon to pass through the atmosphere a sufficient distance to permit the same to solidify into finely divided particles before striking the briquette mixture, whereby the finely divided particles are mixed with the briquetting material, forming the briquetting material into briquettes at a temperature below the melting point of the hydrocarbon, and raising the temperature of the briquettes above the melting point of the hydrocarbon to melt the finely divided particles of the hydrocarbon in the briquettes to waterproof the same.

JOHN A. ERICKSON.